

Dec. 25, 1956

F. K. BLOOM ET AL

2,775,520

COLD-STAMPED ARTICLES

Filed Nov. 5, 1951



INVENTORS

Fredrick K. Bloom  
William C. Clarke, Jr.

BY

THEIR ATTORNEY

# United States Patent Office

2,775,520

Patented Dec. 25, 1956

1

2,775,520

## COLD-STAMPED ARTICLES

Fredrick K. Bloom and William C. Clarke, Jr., Baltimore, Md., assignors to Armco Steel Corporation, a corporation of Ohio

Application November 5, 1951, Serial No. 254,923

### 2 Claims. (Cl. 75—125)

Our invention relates generally to the production of cold-stamped austenitic chromium-nickel stainless steel articles such as table flatwear, displaying coined or stamped surface configuration, and this of desired intricate detail.

Among the objects of our invention is the production of coined or embossed metal products, of which table flatwear is illustrative, of any desired intricacy or ornamentation in surface design from austenitic chromium-nickel stainless steel sheet metal stock in direct and positive manner by cold-working technique without necessity of intermediate anneal and in the absence of appreciable work-hardening, which products conform closely to required sharpness and refinement of surface and finish detail and ornamentation with close, predictable and reproducible adherence to pattern and dimensions, with minimum wear and long useful life of the stamping and coining dies and with minimum investment in plant and labor, the products thus produced having pleasing lustrous surface appearance and detail together with high resistance to corrosion.

Other objects and advantages attending the practice of our invention, in part will be obvious and in part pointed out during the course of the following description, taken in the light of the accompanying drawing.

In the drawing, wherein we illustratively disclose one embodiment of our invention, there is shown a teaspoon having a pattern embossed on its handle.

As conducive to a clearer understanding of certain aspects of our invention, it may be noted that the austenitic chromium-nickel stainless steels possess many desirable characteristics including illustratively, nice surface appearance, ready susceptibility to high polish with lustrous finish, high resistance to corrosion, its non-magnetic qualities and the like. Unfortunately, however, these stainless steels tend to work-harden under cold-stamping, cold-coining or cold-embossing operations at a much steeper rate than do the straight chromium steels. Perhaps this is due to phase-transformation brought about by cold-working, whereby part of the metal is converted from an austenitic to a martensitic phase, thereby becoming more stable and harder. Be that as it may, and regardless of the explanation, the austenitic chromium-nickel stainless steels are found to work-harden at distressingly high rates, a circumstance which drastically limits the number and variety of cold-stamped, cold-coined, or cold-embossed articles which may be produced from these steels.

It has heretofore been observed that in the most common grades of the austenitic chromium-nickel stainless steels, say the 18—8 chromium-nickel grade, the detrimental work-hardening phenomenon is diminished to a certain extent upon substantial increase of the nickel content. A somewhat similar result is had by increasing the manganese content, or by replacing part of the nickel with manganese. Thus, in certain instances of cold-working, current practice has been to increase the nickel content of the conventional 18—8 chromium-nickel alloy by about 3%; to say, 18—11 chromium-nickel. While the steels thus produced, when viewed from a comparative aspect, and when contrasted with the known and available stainless steels, display substantially reduced work-

2

hardening properties, yet they do not by any means fully satisfy the many problems encountered in actual practice. Quite on the contrary, the rate of work-hardening had in cold-stamping, cold-coining and cold-embossing these increased nickel steels still remains so high, even though materially improved over existing steels, as to remain a definite limitation of the production of cold-stamped, cold coined and cold-embossed austenitic stainless steel products.

One of the important factors in the connection noted is the severe wear of the cold-forming dies. Another is the extent to which the coining, stamping and embossing operations may be conducted with reasonable power requirements and size of forming dies. In short, it may be said that the rapid work-hardening of the austenitic alloys has severely limited, except for but comparatively simple patterns, the use of these stainless steels in the production of embossed flatwear such as forks and spoons.

Our invention is directed to alleviating the aforementioned difficulties and to produce stamped, embossed or coined austenitic chromium-nickel stainless steel articles in much more effective manner than has hitherto been possible.

Accordingly, an important object of our invention is to minimize the aforementioned difficulties heretofore confronting the art in simple, practical and successful manner, and at the same time to provide both a variety of austenitic chromium-nickel stainless steel articles, and a method of producing the same, of which articles flatwear is illustrative, cold-stamped, cold-coined, or cold-embossed in direct manner from annealed metal stock, in the substantial absence of intermediate anneal, to a high degree of surface or edge detail or both, and this without appreciable wear of the simple forming equipment required and while maintaining pleasing and lustrous surface finish characteristic of the metal, with high resistance to corrosion, and with non-magnetic qualities, together with low cost and investment in both plant, equipment and labor.

Briefly, we have found that by the addition of a small amount of copper to the known austenitic chromium-nickel stainless steels of say the 18—8 chromium-nickel grade, startling results are achieved in lowering the rate of work-hardening. The addition of copper is observed to be much more effective than an increase in either the nickel or manganese content of the alloy, or both.

The surprising character of the result had is brought into bold relief when it is considered that while copper has heretofore been added to steels for a variety of purposes, it has never heretofore been added to selected steels, and in such amount, as to achieve the results presently obtained.

Thus, illustratively, copper has heretofore been added to steels to increase the corrosion resistance displayed to reducing acids. It has been used to promote physical strengths at high temperatures. It has been added to increase the precipitation-hardening properties. As suggested hereinbefore, however, copper has never heretofore been added to the austenitic chromium-nickel stainless steels in proper amount to bring about appreciable and important decrease in the rate of work-hardening had in cold-stamping, cold-coining, cold-embossing and like operations, attended by important decrease in ultimate tensile strength and with appreciable increased ductility.

In point of fact the phenomenon presently observed is somewhat contrary to what would be theoretically anticipated because it is known that when copper is added to nickel, the metal is hardened and, in addition, tends to work-harden at a faster rate.

We have found, however, and as stated heretofore, that

upon the addition of copper in proper amount to austenitic chromium-nickel stainless steels, increased ductility is imparted, initial hardness is slightly reduced, and the rate of work-hardening also reduced. The tendency of the copper addition to produce a detrimental red-shortening effect is of but little moment. Complete fabrication to finish dimensions and surface is possible through direct, cold-working operations, without intermediate anneal.

We have found that a broad range of composition well suited for the production of cold-stamped, cold-embossed or cold-coined products according to our invention is as follows, carbon up to .15%, manganese up to 15%, chromium 10% to 25%, nickel 7% to 20%, copper 1.0% to 6.0%, and remainder iron.

The carbon is kept within such practical limits as to prevent excessive embrittlement. Moreover, the chromium and nickel ingredients are present in sufficient quantities to range from the border-line case to the full austenitic range. The copper is present in sufficient quantities to bring about the desired diminished work-hardening qualities, while the manganese is present in partial substitution for the nickel, and to impart to the austenitic steel that certain, comparatively slight degree of ductility characteristic of that alloying additive.

Inasmuch as the stamping, embossing or coining operations are substantially ones involving the exertion of compressive stresses, certain cold-compression tests which we have undertaken serve to illustrate the marked advantages attendant upon the addition of copper. These results are expressed in terms of the total work required to deform the various samples. The results thus achieved are set forth in the following table:

Table I

| Heat No. | C    | Cr    | Ni    | Cu   | Cold Hardening Work Factor $\times 1,000 \text{ ft./lbs. per cu. in.}$ |
|----------|------|-------|-------|------|------------------------------------------------------------------------|
| 1        | .068 | 17.70 | 6.56  | —    | 152                                                                    |
| 2        | .032 | 17.46 | 6.00  | 4.11 | 88                                                                     |
| 3        | .067 | 17.43 | 8.06  | —    | 133                                                                    |
| 4        | .063 | 17.39 | 8.04  | 3.04 | 79                                                                     |
| 5        | .075 | 17.02 | 10.15 | —    | 109                                                                    |
| 6        | .067 | 17.17 | 9.98  | 3.04 | 81                                                                     |
| 7        | .060 | 17.83 | 9.98  | 4.91 | 76                                                                     |

It is evident upon considering the foregoing table that the addition of important quantities of copper to either the 18-6, 18-8, or 18-10 grades of austenitic chromium-nickel stainless steel are all accompanied by important decrease in the cold-work-hardening factor. Additionally, and having reference to the 18-10 grade, an increase in copper content from 3% to 5% is accompanied by a further decrease in the work-hardening factor.

While not so important in establishing the suitability of copper-containing austenitic chromium-nickel stainless steels in the production of embossed, stamped or coined stainless steel flatware, nevertheless a general indication of the lowered rate of cold-work-hardening is given by the decrease in the ultimate strength after cold-drawing which is had with the copper addition. This is indicated in the following table:

Table II

| Heat No. | C   | Cr    | Ni    | Cu   | Ult. Tensile Str. (1,000 p. s.i.) after cold-drawing from annealed condition |     |     |     |     |   |
|----------|-----|-------|-------|------|------------------------------------------------------------------------------|-----|-----|-----|-----|---|
|          |     |       |       |      | 0%                                                                           | 20% | 40% | 60% | 75% | — |
| 1        | .05 | 18.85 | 9.42  | —    | 78                                                                           | 120 | 165 | 212 | 246 |   |
| 2        | .05 | 18.17 | 11.42 | —    | 82                                                                           | 117 | 152 | 187 | 212 |   |
| 3        | .05 | 18.92 | 12.77 | —    | 75                                                                           | 113 | 150 | 187 | 212 |   |
| 4        | .03 | 18.16 | 13.56 | 3.10 | 75                                                                           | 95  | 122 | 145 | 152 |   |

From a consideration of Table II it will be seen that with fairly constant carbon content, an increase of the nickel content within the austenitic range is accompanied by decreased ultimate tensile strength, and increased ductility. Similarly, upon the addition of an important amount of copper, say 3%, to the 14-14 chromium-nickel grade, further and very marked decrease in ultimate tensile strength, and consequent increase in ductility, is had upon cold-drawing.

10 The single view of the drawing effectively depicts the pleasing ornamentation which can be achieved, the intricate surface detail made possible being shown at 10, while the pleasingly milled edge is shown at 11. Practically any design which may be desired can be effectively 15 produced in accordance with the practice of our invention.

We have found that perhaps that range of alloy composition best suited for most satisfactory results is carbon .10% maximum, manganese .50% to 2.00%, chromium 20 10% to 20%, nickel 10% to 15%, copper 2.0% to 5.0%, and remainder iron.

In this composition we maintain the silicon content within the normal range. While phosphorus and sulfur are normally maintained low, that is, not exceeding about 25 0.04% phosphorus and 0.03% sulfur (see Metals Handbook, 1948 edition, A. S. M. Cleveland, Ohio, page 563), we permit a range up to say about 0.40% where some machining is required in addition to the embossing steps. Selenium up to 0.40%, where desired, may be 30 added for this purpose. And where we desire to stabilize the carbon we sometimes include columbium or titanium in the minimum amounts, respectively, of 8 x percent C and 4 x percent C. The addition of up to 4% molybdenum is found to improve corrosion resistance. None of 35 these various additions seems to adversely affect the stamping, coining or embossing properties.

By the practice of our invention we produce, in highly satisfactory manner, stamped, coined or embossed products, such as ornamented stainless steel flatware, spoons and forks. This objective is achieved in simple and 40 positive manner, directly from stainless steel sheet or strip stock. Necessity for intermediate anneal is effectively eliminated. At all times the cold-hardening rate is retained within effective limits, and the forming equipment, including shaping and stamping dies, display long useful life. At the same time many advantages of stainless steel are availed of fully and effectively including non-magnetic properties, pleasing and lustrous surface appearance, high resistance to corrosion, and the like.

50 All these, as well as many other highly practical advantages tend upon the practice of our invention.

It is apparent from the foregoing that once the broad aspects of our invention are disclosed, many embodiments thereof will readily occur to those skilled in the art, and all falling within the ambit of our disclosure. 55 Accordingly, we intend our present disclosure to be considered solely as illustrative, and in no sense limitative.

We claim as our invention:

1. Cold-stamped and machined stainless steel articles 60 analyzing approximately up to 0.15% carbon, up to 15% manganese, from about 10% to about 25% chromium, from about 7% to about 20% nickel, from about 1.0% to about 6.0% copper, one element of the group consisting of about 0.04% to 0.40% phosphorus and about 65 0.03% to 0.40% sulfur, and remainder iron.

2. Cold-stamped and machined stainless steel articles 70 analyzing approximately, up to 0.10% carbon, about 0.50% to about 2.00% manganese, about 10% to about 20% chromium, about 10% to about 15% nickel, about 2.0% to about 5.0% copper, one element of the group consisting of about 0.04% to 0.40% phosphorus and about 0.03% to 0.40% sulfur, and remainder iron.

## References Cited in the file of this patent

## UNITED STATES PATENTS

|           |           |                |
|-----------|-----------|----------------|
| 1,285,852 | Watrous   | Nov. 26, 1918  |
| 2,066,085 | Whistler  | Dec. 29, 1936  |
| 2,523,000 | Defranoux | Sept. 19, 1950 |

## FOREIGN PATENTS

|         |               |               |
|---------|---------------|---------------|
| 437,592 | Great Britain | Oct. 23, 1935 |
|---------|---------------|---------------|

## OTHER REFERENCES

Alloys of Iron and Chromium, High Chromium, vol. 2, pages 433 and 434. Edited by Kinzel and Franks. Pub. in 1940 by the McGraw-Hill Book Co., New York, N. Y.

Die Design and Diemaking Practice, 3rd edition, pages 901-904. Edited by Jones. Pub. in 1951 by the Industrial Press, New York, N. Y.